

## UNITED STATES PATENT OFFICE.

JAMES BADDILEY, PERCY CHORLEY, AND CARLTON BUTLER, OF MANCHESTER, ENGLAND, ASSIGNORS TO BRITISH DYESTUFFS CORPORATION LIMITED, OF MANCHESTER, ENGLAND, A COMPANY OF GREAT BRITAIN AND IRELAND.

## PROCESS FOR DYEING ARTIFICIAL SILK.

No Drawing. Application filed April 2, 1927, Serial No. 180,610, and in Great Britain June 4, 1926.

According to this invention, regenerated cellulose silks, such as viscose silk, are dyed with the secondary disazo dyestuffs obtained by coupling amino-salicylic acids or their homologues, hereafter referred to as amino-*o*-hydroxy-carboxy acids of the benzene series, with the usual middle components, further diazotizing and combining with the so-called sulphonated 1:8-di-substituted 10 naphthalene derivatives as end components. The said components are 1:8-dihydroxy-naphthalene sulphonic acids, 1:8-amino-naphthol-sulphonic acids and N-substituted derivatives of the latter. Secondary disazo 15 compounds are those obtained by the action of a diazoazo compound on an amine or a phenol. The use of dyestuffs of the present type for dyeing chrome mordanted wool and for chrome printing has long been known, 20 but we have now made the entirely unexpected discovery that the dyestuffs have a good affinity for regenerated cellulose silks and possess the valuable property of giving level dyeings on these fibres.

25 The regenerated cellulose silk fibres have hitherto given considerable difficulty in dyeing owing to the fact that they are liable to possess an uneven affinity for dyestuffs, which causes the dyeings obtained to be uneven. This difficulty is encountered particularly when it is desired to dye the fibre in blue and green shades. The shades which we obtain are blue, green and black and are very level, and our discovery is therefore of 30 considerable technical value.

The aminosalicylic acids we use may be either 5-aminosalicylic acid



40 or its 1:2:3 isomer, or the technical mixture of these two isomers, and the homologues of any of these may be used. As middle components, there may be used  $\alpha$ -naphthylamine, 1-amino-2-naphthol ethers, 45 1-naphthylamine-6- or 7-sulphonic acids, 1-amino-2-alkyloxy-naphthalene-6- or 7-sulphonic acids, meta-amino-para-cresolmethyl-ether, amino-hydroquinone-dimethyl ether and the like.

50 The fibre is dyed in the usual way, suitable conditions being as follows, but we do not limit ourselves to the conditions here described. The parts indicated are by weight.

A dyebath is made up from 3000 parts of 55 water, 20 parts of Glauber's salt, 2 parts of soap and one part of the secondary disazo dye obtained by combining 5-aminosalicylic acid with 1-amino-2-naphthol ethyl ether, rediazotizing and combining with 1:8-dihydroxynaphthalene-4-sulphonic acid. 100 parts of the regenerated cellulose silk are entered into the bath at about 30° C., the 60 bath is then heated to about 90° C. and dyeing allowed to proceed for about one hour. The silk is then removed, rinsed and dried. The resulting dyeing is a level bright green shade.

The following table contains other examples of the shades which can be obtained by our invention:

| Secondary disazo dyes from:-            |                          |                                                 | Shade on viscose silk | 75 |
|-----------------------------------------|--------------------------|-------------------------------------------------|-----------------------|----|
| First component                         | Middle component         | End component                                   |                       |    |
| 5-aminosalicylic acid.                  | $\alpha$ -naphthylamine. | 1:8-aminonaphthalene-3:6-disulphonic acid.      | Greenish-black.       |    |
| Ditto.....                              | ditto.....               | 1:8-dihydroxynaphthalene-3:6-disulphonic acid.  | Blue-black.           |    |
| Ditto.....                              | ditto.....               | 1:8-aminonaphthalene-2:4-disulphonic acid.      | Blue-black.           | 80 |
| Aminosalicylic acid. Technical mixture. | m-amino-p-cresol.        | 1:8-dihydroxynaphthalene-4-sulphonic acid.      | Blue.                 |    |
| Aminosalicylic acid. Technical mixture. | $\alpha$ -naphthylamine. | 1:8-dihydroxynaphthalene-4-sulphonic acid.      | Blue.                 |    |
| Ditto.....                              | ditto.....               | 1-acetamino-8-naphthalene-3:6-disulphonic acid. | Blue-black.           | 85 |
| Ditto.....                              | Cleves acid (mixed).     | 1:8-dihydroxynaphthalene-4-sulphonic acid.      | Greenish-blue.        |    |
| p-amino- <i>o</i> -cresotinic acid.     | $\alpha$ -naphthylamine. | 1:8-dihydroxynaphthalene-3:6-disulphonic acid.  | Blue.                 | 90 |
| o-amino-p-cresotinic acid.              | ditto.....               | 1:8-dihydroxynaphthalene-3:6-disulphonic acid.  | Grey-blue.            |    |

What we claim and desire to secure by Letters Patent is:-

1. The process of dyeing which comprises dyeing regenerated cellulose silks with the secondary disazo dyestuffs which can be made by combining amino-*o*-hydroxy-carboxy acids of the benzene series with the usual middle components, further diazotizing and combining with a sulphonated 1:8-di-substituted naphthalene derivative.
2. The process of dyeing which comprises dyeing regenerated cellulose silks with the secondary disazo dyestuffs which can be

made by combining amino-o-hydroxy-carboxy acids of the benzene series with the usual middle components, further diazotizing and combining with a sulphonated 5 1:8-dihydroxynaphthalene.

3. The process of dyeing which comprises dyeing regenerated cellulose silks with the secondary disazo dyestuffs which can be made by combining amino-o-hydroxy-10 carboxy acids of the benzene series with the usual middle components, further diazo-

tizing and combining with a 1:8-dihydroxy-naphthalene-4-sulphonic acid.

4. As new industrial products, regenerated cellulose silks dyed by the process 15 of claim 1.

In testimony whereof we affix our signatures.

JAMES BADDILEY.  
PERCY CHORLEY.  
CARLTON BUTLER.